

Jan. 19, 1965

G. C. RIEGGER ET AL.

**3,166,388**

## SANDPAPER

Filed Jan. 23, 1962

Diagram illustrating the layers of a sanding block:

- Making Varnish layer 8
- Backing 6
- Abrasive grits 9
- Barrier layer-Vinyl 7

Fig. 2.

12 13 11 14 12  
11 13 12  
11 14 12  
14 11 13 11  
12 11 14 13 11  
13 11 14 13

INVENTORS:  
GEORGE C. RIEGER  
RICHARD M. SMITH  
BY  
*Charles A. Harris*  
ATTORNEY

1

3,166,388  
SANDPAPER

George C. Riegger, Miami Beach, Fla., and Richard M. Smith, New Brunswick, N.J., assignors to Johnson & Johnson, a corporation of New Jersey

Filed Jan. 23, 1962, Ser. No. 169,704

9 Claims. (Cl. 51—296)

The present invention relates to paper backed abrasive papers, more particularly to such papers of the type known as sandpapers.

This application is a continuation-in-part of my pending application, Serial No. 829,629, filed July 27, 1959, and now abandoned.

Conventionally, sandpapers have been made in the form of a laminate comprising a paper backing, a barrier material, and a layer of hard tough material having a layer of grits imbedded therein. The hard tough material generally is of a type known in the trade as making varnish. In conventional sandpapers crack resistance in use depends for the most part upon the layer of varnish holding the grits with the result that when the varnish cracks the backing may crack along the same line shortly thereafter. When the cracks in the varnish occur in folding the sandpaper, this problem is accentuated because the backing, itself, is stressed directly and often is abraded along the fold line. In wet sanding the paper tends to fail due to its decreased tensile strength and abrasion resistance when wet.

The present invention contemplates a sandpaper in the form of a laminate of the above general type, but which possesses superior internal strength, fold endurance, crack resistance, wet and dry tensile strength and wet abrasion resistance.

Sandpapers according to this invention comprise a reinforced paper backing, a barrier material, a layer of making varnish and a layer of abrasive grits imbedded in the making varnish. The barrier material may be in the form of a barrier layer of flexible material which only partly penetrates into one side of the backing, or it may be in the form of flexible rubbery solids which penetrate into and partially fill the voids in the paper backing throughout its thickness. When the term "rubbery" is used hereinafter in this application with reference to a material, it refers to the physical, not the chemical, properties thereof. In either case, the barrier material must be (1) flexible, (2) compatible with both the (a) paper backing and the (b) making varnish layer so as to bond to both of them, and (3) capable of preventing the making varnish from penetrating substantially into the backing.

The backing is a relatively heavy paper normally having a basis weight between about 40 and 150. However, lower basis weight backings may be advantageous in certain types of abrasive papers according to this invention. When used in this application, basis weight shall be expressed in pounds per ream of 480 sheets 24 inches wide and 36 inches long. Backings according to this invention comprise a web or network of overlapping crossing kraft-type woodpulp fibers and a multiplicity of relatively large flexible and tough thermoplastic reinforcing members distributed substantially uniformly throughout the web in bonding relation with the woodpulp fibers. The woodpulp fibers are arranged in overlapping crossing relation with one another so as to define a multiplicity of minute interstices between them. The relatively large reinforcing members define a corresponding multiplicity of spaces between the members in the web. The average distance across the spaces between the reinforcing members is considerably greater than the average distance across, or the size of, the relatively minute interstices between the woodpulp fibers so that several of these inter-

2

stices between the woodpulp fibers so that several of these interstices generally are located in each of the spaces between the reinforcing members.

The woodpulp fibers are relatively small when compared with the reinforcing members, i.e., the woodpulp fibers are in the range of about 0.04 to 0.4 mil in thickness and about 0.4 to 0.8 mil in width, and are less than  $\frac{1}{4}$  inch in length normally within the range of about 80 to 240 mils, while the reinforcing members are in the range of 1 to 35 mils in cross dimension and may be as long as an inch or more, depending upon shape factors such as their length-to-width ratio. For instance, if they are in the form of rods having a more or less circular cross section and a length-to-width ratio of 2 to 1, normally over 10 to 1 or more, their cross dimensions may fall within the range of about 1 to 5 mils; and they may be between about  $\frac{1}{32}$  and 1 inch or over in length, although rods below about  $\frac{1}{4}$  inch in length may be preferred. However, when the length-to-width ratio of the reinforcing members is decreased until length and width become more nearly equal to each other and the members are in the form of granules, the cross dimension of the reinforcing members may be between about 5 and 35 mils.

In a given product according to this invention, the sizes of the reinforcing members and the woodpulp fibers are of different orders of magnitude, i.e., the individual reinforcing members are at least about 5, preferably 10 or more, times larger in cross-sectional area than the individual woodpulp fibers. Thus, even if equal proportions of the woodpulp fibers and reinforcing members are used, the above-described relationship exists wherein the spaces between the reinforcing members are considerably larger than the interstices between the woodpulp fibers. However, the reinforcing members are applied in the web in certain definite proportions which contribute to the desired structure. Normally, the over-all weight of the reinforcing members with respect to the dry woodpulp fiber solids falls within the range of about 5 to 30 percent, although as little as 2 or 3 percent and as much as 60 percent or more of the reinforcing members by weight may be used with desirable results for certain applications.

The woodpulp fibers in the spaces between the reinforcing members in the backings of this invention are bonded to one another by hydration bonds formed between the fibers. According to one embodiment of the invention, rubbery binder solids portions may be present in the backing, distributed substantially uniformly throughout the web of woodpulp fibers to cooperate with the hydration bonds between the woodpulp fibers to bond the fibers together. Generally speaking, if the amount of rubbery binder solids in the backing is increased, the internal strength of the backing also will be increased. However, it is an important advantage of this invention that backings may be provided which when incorporated in the above-described sandpaper laminate provide an abrasive paper which possesses superior internal strength, fold endurance, crack resistance, wet and dry tensile strength and wet abrasion resistance whether or not the rubbery binder solids portions are present. The rubbery binder solids portions may be applied to backings according to this invention in different amounts depending upon the internal strength desired and cost considerations. If cost is a prime factor, the rubbery binder solids may be dispensed with or applied in relatively minor amounts. However, when the making varnish, or grit bonding layer, is a rubber latex, for instance, the rubbery binder solids may act as the barrier material if present in the backing in sufficient amount, in which case said solids perform a double function, i.e., to increase the internal strength of

the backing and to prevent penetration of the backing by the making varnish.

It is believed that the superior fold and crack resistance of abrasive papers according to this invention is due largely to the increased strength and flexibility of the paper backing. In general, the more flexible the backing, the less it is likely to be affected adversely by folding of the sandpaper or cracking of the making varnish layer.

The structure of the fabric of this invention will be explained and may be better understood by reference to the following drawings wherein:

FIGURE 1 is an enlarged schematic view in elevation of a portion of an abrasive paper according to this invention;

FIGURE 2 is an enlarged schematic plan view of an abrasive paper according to this invention as one embodiment may appear; and

FIGURE 3 is a greatly enlarged schematic sectional view of a portion of FIG. 1.

Referring to the drawings, there is shown an abrasive paper comprising a reinforced paper backing 6, a barrier layer 7, a layer 8 of making varnish and a multiplicity of grits 9 embedded in the making varnish layer 8. In the backing 6, relatively short and small woodpulp fibers 11 are arranged in overlapping crossing relation with one another so as to form a multiplicity of interstices 12 between them. The woodpulp fibers are bonded together by hydration bonding between the fibers 11 where they cross in contact with one another, as well as by a multiplicity of relatively large rod-shaped flexible and tough thermoplastic polymeric reinforcing members 13 distributed substantially uniformly throughout the web.

Each of the reinforcing members 13 bonds a large number of woodpulp fibers 11 which pass through or into contact with the member. As shown most clearly in FIG. 3, the individual reinforcing members 13 entrap a number of adjacent or contiguous woodpulp fibers 11 in the plane of the web and perpendicular thereto, or through the thickness of the web. The woodpulp fibers 11 are held firmly in the individual reinforcing members 13 since the woodpulp fibers passing through each member 13 are in contact with the material of the reinforcing member along a high proportion of the length of the woodpulp fibers 11.

The reinforcing members 13 define a multiplicity of spaces 14 between them; and the average distance across the spaces is considerably greater than the average distance across the interstices 12, or the size of the interstices, formed between interlacing woodpulp fibers 11. Thus, several of these interstices 12 generally are located in each of the spaces 14 formed between the reinforcing members 13.

In a sense, the web is "interrupted" by the reinforcing members 13 so as to form a multiplicity of web "islands" corresponding to the web areas in the spaces 14 between the reinforcing members 13, which are joined together by the reinforcing members. Continuing this analogy, the islands are formed by the woodpulp fibers 11 which are bonded together to form a connected network structure in the spaces 14. The reinforcing members 13 defining the islands may be compared to hinges between islands which provide elements of flexibility scattered throughout the web structure. It is believed that the hinged island structure just described may contribute to the improved flexibility of backings of this invention, although other factors such as fiber orientation also may affect flexibility.

In forming backings according to this invention, it is preferred to distribute the reinforcing members in the web during the papermaking step. Normally, this step involves beating the woodpulp fibers to hydrate them to the extent necessary to form the desired hydration bonds in the backing and then distributing them in water to form an aqueous slurry of woodpulp fibers and mixing the

proper proportion of thermoplastic reinforcing members with the woodpulp fibers in the slurry until they are distributed substantially uniformly in the slurry and intimately intermingled with the woodpulp fibers. The slurry is then drained through some sort of collecting means for making paper such as a Fourdrinier wire, a drum screen, a hand sheet mold, or the like to form a paper web. After drying and pressing as is conventional in papermaking, heat and pressure are applied to the web containing the reinforcing members in such a way as to soften and preferably fuse the thermoplastic reinforcing members and press them through the thickness of the web so that they entrap a large number of woodpulp fibers. Temperature and pressure are controlled carefully so that the material of the reinforcing members does not flow too freely and cause the members to lose their shape. For instance, if temperature is too high, under certain pressures surface tension may cause the material in the reinforcing members to "ball up"; and of course if pressure is too high, it will squeeze the reinforcing members and flatten them out to too great an extent. It is inevitable in this process that the reinforcing members be flattened to a certain extent, and allowance can be made for this. Thus, the cross dimension of the reinforcing members in the resulting fabric may be as great as twice that of the rods or granules from which they are formed, although the increase in cross dimension due to the application of heat and pressure during the bonding of the reinforcing members normally is not this great.

If it is desired to distribute rubbery binder solids portions in the backing, the woodpulp fibers need not be beaten prior to formation of the slurry or they may be beaten to some extent depending upon the properties desired in the finished product. After the bonds between the reinforcing members and the woodpulp fibers have been formed and the web has been allowed to cool to permit the bonds to become set, the rubbery binder solids may be applied thereto. Normally, this is accomplished by impregnating the web with an aqueous dispersion of a natural or synthetic rubbery latex, or by impregnating it with a natural or synthetic rubber composition deposited from solution in a volatile organic solvent. These methods are taught in United States Patents 2,726,967 and 2,236,527, respectively.

Woodpulp, the fibers of which are suitable for use in producing backings in accordance with this invention, include relatively long fiber kraft-type pulps, such as Duracel pulp. As mentioned hereinbefore, the individual woodpulp fibers are in the range of about 0.04 to 0.4 mil in thickness and about 0.4 to 0.8 mil in width, and generally are less than about 1/4 inch, say about 80 to 240 mils, in length. From the above, it is apparent that the woodpulp fibers are somewhat flat, or ribbon like, in shape. They may be more or less straight or somewhat curled and kinked as may result from being subjected to treatment such as described in United States Patent 2,516,384 to provide curled fibers.

The relatively flexible and tough thermoplastic reinforcing members of this invention preferably are selected from among a number of long-chain polymeric materials which form flexible and tough solid granules or rods. Nylon 6 comprising polycaprolactam gives particularly good results when used as the material for the reinforcing members of this invention. Other materials, which may be employed for the reinforcing members, include nylon 11 such as sold under the trademark "Rilsan" by Organico, S.A., of France, saran, polyamides other than nylons 6 and 11, polyvinyl chloride, polyethylene, polyurethane, polystyrene, polyvinylidene cyanide, plasticized cellulose acetate, plasticized ethyl cellulose, and the like.

The size of the reinforcing members may vary over a wide range. If the reinforcing members are in the shape of rods, prior to fusing, they normally would fall within the range of about 6.5-100 denier, corresponding to about 0.0005-0.004 inch in diameter prior to fusing

for the flexible and tough thermoplastic materials of this invention, and  $\frac{1}{32}$  to 1 inch in length. Preferably, the rods would be between about 10 and 60 denier, corresponding to about 0.0012-0.0034 inch in diameter prior to fusing, and in the neighborhood of  $\frac{1}{4}$  inch or less in length. If the reinforcing members of this invention are in the shape of granules, prior to fusing, they normally would be of such a size that 70 percent of the granules would not pass through a 200 mesh screen. Preferably, the majority of the particles are of a size that would not pass through a 100 mesh screen. This means that generally speaking the average granule size will be within the range of about 0.004-0.015 inch in diameter prior to fusing. Rods and granules outside the indicated ranges may be used provided that they are at least about 5, preferably 10 or more, times larger in cross-sectional area than the woodpulp fibers with which they are used.

The rubbery solids portions may be supplied from various natural and synthetic elastomeric materials, or mixtures of an elastomeric component with a thermosetting component, such as are described in United States Patents 2,848,105 and 2,848,355. As mentioned hereinbefore, the elastomer, or elastomeric mixture, may be in the form of an aqueous dispersion of a synthetic rubbery latex or a natural or synthetic rubber composition in solution in a volatile organic solvent. Suitable synthetic rubbery latices may comprise polymers of butadiene and other conjugated dienes and their homologues, and copolymers and tripolymers based thereon, vinyl chloride polymers, copolymers of vinyl chloride with other materials such as vinyl acetate and vinylidene chloride, chloroprene rubber and various other similar elastomeric polymers. Copolymers of butadiene and unsaturated nitriles, such as acrylonitrile and the like, have been found to be particularly suitable for this purpose.

Before application to the fibrous web, the rubbery binder solids may be in the form of relatively small particles ranging in size from about 0.004 to 0.2 mil in cross section, preferably not above about 0.04 mil, normally having a length-to-width ratio in the neighborhood of 1:1. As the rubbery binder is applied to the web formed by the woodpulp fibers 11 and the reinforcing members 13, rubbery binder solids portions, not shown, are formed between the woodpulp fibers. The rubbery binder material may remain in the form of the original relatively small latex particles in which it is deposited. However, as the amount of the rubbery binder in the web is increased, the original latex particles tend to join one another and form an at least partially continuous rubbery matrix with the rubbery binder solids portions connecting the woodpulp fibers in the areas 14 between the binder members 13 being in the form of agglomerates which may be somewhat film-like in character. As the concentration of the rubbery binder solids portions is increased, the deposited binder material becomes less particle-like and more like a continuous matrix in nature.

Abrasive papers according to this invention may be formed from the above-described backings as follows. If the rubbery binder solids are present in the web in sufficient amount (say about 10% by weight of the dry fibers) to act as a barrier material, the web containing the rubbery solids may be coated directly with a layer of making varnish based on a rubber latex adapted to be vulcanized in-situ on the web. In such a case the barrier material substantially prevents further penetration of the backing by the making varnish and is compatible with the backing and the making varnish layer so as to bond to both of them.

When a hard and tough making varnish such as the resin reaction product of a melamine aldehyde and China-wood oil is to be used, normally the backing is coated with a flexible barrier material such as polyvinyl chloride plasticized with a copolymer based on butadiene which forms a layer on one side of the backing which will prevent the making varnish from penetrating into the

backing and is compatible with both the backing and the making varnish for bonding purposes. In this case, the main purpose of the barrier layer is to prevent the hard and tough making varnish from penetrating into the paper backing and rendering it hard and brittle. Various materials can be used for this purpose which are flexible and capable of resisting penetration by the making varnish and capable of providing the required bonding between the varnish and the backing. The making varnish, itself, may be applied in two layers; the first being applied directly to the surface of the impregnated backing or the barrier layer, as the case may be, and the second being applied after the grits have been seated in the first layer of making varnish. This second layer sometimes is called the sand-size. As indicated above, the grits normally are applied in a layer to the first layer of making varnish while the varnish layer still is soft so that the grits are imbedded in the varnish as shown in FIG. 1 of the drawings. Conventional sand, or silicon carbide, grits or other abrasive grits of the type normally used in this general type of product may be employed. The sandsize is applied in a layer sufficiently thick to assure that the grits will be held firmly in the making varnish after the varnish is dried, and the resulting product then may be dried and cured for several hours at an elevated temperature to bond the grits firmly in the varnish.

As indicated hereinbefore, the barrier material must be (1) flexible, (2) compatible with both (a) the paper backing and (b) the making varnish so as to bond to both of them, and (3) capable of preventing the making varnish from penetrating substantially into the backing. Different barrier materials according to this invention are listed below opposite typical making varnishes with which they may be used.

|       | Barrier Material                | Making Varnish                                                        |
|-------|---------------------------------|-----------------------------------------------------------------------|
| 1.    | Oil compatible glyptal resin... | Resin from reaction product of phenol aldehyde resin and fatty oil.   |
| 2.    | Halogenated rubber...           | Halogenated rubber.                                                   |
| 3.    | Vulcanized rubber...            | Vulcanized rubber.                                                    |
| 4.    | Phenol-aldehyde resin...        | Phenol-aldehyde resin.                                                |
| 5.    | do                              | Urea-aldehyde resin.                                                  |
| 6.    | Vinyl acetal resin...           | Phenol-aldehyde resin.                                                |
| 7.    | Ethyl cellulose resin...        | Do.                                                                   |
| 8.    | Gelatin...                      | p-Phenol sulfonic acid rubber reaction product.                       |
| 45 9. | Plasticized polyvinyl chloride. | Resin reaction product of melamine aldehyde resin and China-wood oil. |

The following examples are illustrative of different embodiments of abrasive papers according to this invention.

#### Example I

A sandpaper backing according to this invention is made from curled Duracel pulp having a Schopper-Riegler freeness of about 750 cc. and 20% by weight of the total mixture of 15 denier nylon 6 rods about  $\frac{1}{16}$  inch long. The above materials are collected on a suitable papermaking screen to form a paper backing about 7.5 mils thick and weighing about 70 pounds per ream. Bonds are formed between the nylon 6 rods and the woodpulp fibers by pressing in a Carver press at 200 pounds per square inch and 425° F. for 10 seconds.

The backing paper is coated on one side with a barrier coat comprising polyvinyl chloride plasticized with a copolymer of butadiene and acrylonitrile (polyvinyl chloride to butadiene-acrylonitrile ratio being about 70:30) to deposit a barrier layer weighing about 6 pounds per ream. After drying, a coating of abrasive grains is applied on top of the barrier coat by the following procedure. About 2.3 pounds per ream of a making varnish comprising the resin reaction product of about 20 parts of melamine-formaldehyde resin and 80 parts of a varnish based on China-wood oil is painted over the barrier coat and about 4.5 pounds per ream of silicon carbide grits are applied thereto while the varnish still is wet. About 3.8

pounds per ream of a sandsize of the same varnish is applied on top of the grits and then dried. The resulting product is cured for 8 hours at 225° F. This procedure is described more fully in Canadian Patent No. 568,647. The final cured product is an inexpensive sandpaper of superior fold endurance, crack resistance, wet and dry tensile strength and wet abrasion resistance.

*Example II*

Another sandpaper backing according to this invention is made from curled Duracel pulp having a Schopper-Riegler freeness of about 820 cc. and 15% by weight of the total mixture of 15 denier nylon 6 rods about  $\frac{1}{16}$  inch long in the same manner as for Example I to form a paper backing about 4 mils thick and weighing about 38 pounds per ream. This paper is treated as described in Example I to form bonds between the rods and the woodpulp fibers. The bonded paper is impregnated with a mixture consisting of about 99.5 parts on a solids basis of a butadiene-acrylonitrile latex and about 0.5 part of the sodium salt of ethylene diamine tetraacetic acid in such way that the total impregnant solids deposited weigh about 10% of the dry fibers in the sheet. The impregnated paper is then formed into a sandpaper laminate in the manner described in Example I to produce an inexpensive sandpaper which possesses superior fold endurance and crack resistance and exhibits internal strength, tensile strength and abrasion resistance when wet slightly greater than that of the paper of Example I on a weight-for-weight basis.

*Example III*

A sandpaper backing is made and impregnated to deposit about 10% by weight of the dry fibers of rubbery binder solids, as described in Example II. The impregnated backing then is coated directly with about 7.5 pounds per ream of a making varnish consisting of a vulcanizable rubber latex adapted to be heat cured at a temperature of about 130° C. The rubbery binder solids in the web prevent the making varnish from penetrating substantially into the backing. While the making varnish is still wet about 4 pounds per ream of silicon carbide grits are applied thereto. The resulting product then is cured for several hours at a temperature above 130° C. to bond the grits firmly in the varnish. The resulting product is a flexible sandpaper of high crack resistance and wet abrasion resistance.

Having now described the invention in specific detail and exemplified the manner in which it may be carried into practice, it will be readily apparent to those skilled in the art that innumerable variations, modifications, applications, and extensions of the basic principles involved may be made without departing from its spirit and scope.

The invention claimed is:

1. An abrasive paper which comprises a reinforced paper backing web, a layer of grit supporting making varnish on one side of said paper with a multiplicity of abrasive grits imbedded in said varnish, and a flexible barrier material preventing the making varnish from penetrating substantially into the backing, said barrier material being compatible with both the backing and the making varnish and bonding the backing to the varnish, said web comprising a continuous network of kraft-type wood-

5 pulp fibers arranged in overlapping crossing relationship with one another so as to define a multiplicity of interstices between them, and a multiplicity of flexible and tough thermoplastic reinforcing members distributed substantially uniformly throughout the web in bonding relation with the wood-pulp fibers, said reinforcing members being between about 1 and 35 mils in cross dimension and at least about five times larger in cross-sectional area than said woodpulp fibers and defining a multiplicity of spaces between said members, the average distance across the spaces between the reinforcing members being considerably greater than the average distance across the interstices between the woodpulp fibers whereby several of said interstices generally are located in each of the spaces between the reinforcing members.

10 2. An abrasive paper according to claim 1, wherein elastomeric binder solids portions are distributed substantially uniformly throughout the web and said solids portions form a multiplicity of bonds between the woodpulp fibers in the individual spaces between the reinforcing members.

15 3. An abrasive paper according to claim 1, wherein said thermoplastic reinforcing members essentially comprise nylon.

20 4. An abrasive paper according to claim 2, wherein said elastomeric binder solids also act as the barrier material and said making varnish comprises a vulcanizable rubber latex.

25 5. An abrasive paper according to claim 1, wherein said barrier material is in the form of a flexible layer between said backing and the making varnish layer bonding the backing and the making varnish to one another, said barrier layer preventing substantial penetration of the making varnish into the backing.

30 6. An abrasive paper according to claim 1, wherein the reinforcing members are present in the web in an amount ranging between about 5 and 30 percent based upon the combined dry weight of the fibers and the reinforcing members.

35 7. An abrasive paper according to claim 6, wherein the reinforced backing web has a basis weight between about 40 and 150.

40 8. An abrasive paper according to claim 1, wherein said reinforcing members are rod-shaped.

45 9. An abrasive paper according to claim 8, wherein said rod-shaped reinforcing members are between about 1 and 5 mils in cross dimension.

References Cited in the file of this patent

UNITED STATES PATENTS

|           |                    |               |
|-----------|--------------------|---------------|
| 2,186,001 | Bartling           | Jan. 9, 1940  |
| 2,236,597 | Hatch              | Apr. 1, 1941  |
| 2,356,866 | Melton et al.      | Aug. 29, 1944 |
| 2,468,853 | Williamson         | May 3, 1949   |
| 2,627,145 | Frigstad           | Feb. 3, 1953  |
| 2,981,615 | Baumgartner et al. | Apr. 25, 1961 |
| 3,014,793 | Schmidlin          | Dec. 26, 1961 |

FOREIGN PATENTS

|         |           |              |
|---------|-----------|--------------|
| 118,147 | Australia | Mar. 2, 1944 |
|---------|-----------|--------------|